# EUROPEAN PATENT SPECIFICATION

(11) **EP 1 501 102 B1**
(45) Date of publication and mention of the grant of the patent: **23.09.2009**
(21) Application number: 04010648.6
(22) Date of filing: 05.05.2004
(51) Int. Cl.: H01B 7/00

(54) **Improved electric cable**
Verbessertes elektrisches Kabel.
Câble électrique amélioré.

(30) Priority: 23.07.2003 IT MI20030349
(43) Date of publication of application: 26.01.2005
(73) Proprietor: Controlcavi Industria S.r.l., 20010 Bernate Ticino (Milano) (IT)
(72) Inventor: Brambilla, Angelo, 20010 Bernate Ticino Milano (IT)
(74) Representative: Cicogna, Franco

## Description

### BACKGROUND OF THE INVENTION

The present invention relates to an improved electric cable conductor.

As is known, electric cables conventionally comprise one or more electric conductors or wires, coated by an insulating material.

The constructional parameters and characteristics of the mentioned conductors, according to reference rules, are divided into Classes, defining their electric, cross-section and diameter characteristics.

The conductor family according to the present invention is referred to Class 2 of the IEC (International Electrotechnical Commission) 60228 rule.

The conductors in this Class are defined as "rigid" and they must comprise a small minimum number of component elementary wires (see the accompanying table).

The stiffness or rigidity characteristic of the conductor is a consequence of the greater diameter of the few elementary individual wires thereof, which, moreover, have a diameter which increases proportionately to the overall cross-section of the conductor itself.

Another required rule to be met is the maximum value of the electric resistance of the conductor.

Vice versa, the above mentioned standard or specification provides, in the Class 5, a conductor for electric cables comprising a high number of small diameter elementary wires, thereby providing the conductor with flexibility properties, but with larger allowed electric resistance values.

It should be pointed out that a less electric resistance value would involve, the conductor cross-section being the same, a larger current capability.

In general, the flexibility of an electric conductor will depend, for each cross-section thereof, on the diameter of the elementary wires and their numbers, so as to meet the standardizing requirements and criteria related to their assembling for providing a reduced diameter of the finished conductor.

### SUMMARY OF THE INVENTION

The aim and objects of the present invention is to provide a flexible conductor of Class 2, by suitably assembling a comparatively high number of small elementary wires, so as to provide said flexible conductor with the desired flexibility characteristics, similar to or better than those of Class 5, but with an electric resistance as that required by Class 2 (and accordingly a larger current flow capability). This is achieved with a flexible electric multiple elementary wire cable according to claim 1.

### BRIEF DESCRIPTION OF THE DRAWINGS

Further characteristics and advantages of the present invention will become more apparent hereinafter from the following drawings and enclosed tables.

It should be apparent that the invention can be made, for each cross-section, by exploiting the most suitable combination of the diameter of the selected elementary wire, in the range shown in the table, the elementary wire number to meet the required electric resistance characteristic, and the adopted assembling technique.

A further characteristic shown in the table is the small diameter of the conductor of the inventive cable with respect to that of an equivalent conventional "rigid" conductor of Class 2 and, more specifically, with respect to that of a related conductor of Class 5.
Figure 1 shows a portion of the electric cable according to the invention, the insulation material being partially removed;
Figure 2 is a view similar to figure 1;
Figure 3 is a view of the cable as cross-sectioned along the plane III-III of figure 2.

### DESCRIPTION OF THE PREFERRED EMBODIMENT

With reference to the number references of the above mentioned figures, the insulated flexible cable according to the invention has been generally indicated by the reference number 1, and comprises a conductor 2 electrically insulated at 3.

The conductor 2 of the insulated electric cable 1 according to the invention is constructed according to the electric and minimum wire number characteristics of Class 2 but, owing to the large number of said wires, which have a small diameter, has a flexibility equal to or better than that of the conductors of Class 5, for some cross-sections of the conductor, as shown in the enclosed Table.

The table shows, for conductors of red copper wires and tinned copper wires data related to parameters characterizing the inventive cable, for the disclosed cross-sections:

**TABLE**

| | **CHARACTERISTICS OF THE INVENTIVE FLEXIBLE ELECTRIC CABLE** | | | |
|---|---|---|---|---|
| | 1 | | 2 | 3 |
| Cross Section of the conductor [mm²] | Maximum electric resistance [at 20°C] of the conductor | | Diameter of the elementary wires [mm] | Maximum diameter of the conductor [mm] |
| | Red Copper [Ohm/km] | Tinned Copper [Ohm/km] | | |
| 6 | 3.08 | 3.11 | 0.30 ÷ 0.90 | 3.2 |
| 10 | 1.83 | 1.84 | 0.30 ÷ 0.90 | 3.8 |
| 16 | 1.15 | 1.16 | 0.30 ÷ 0.90 | 4.9 |
| 25 | 0.727 | 0.734 | 0.30 ÷ 0.90 | 6.1 |
| 35 | 0.524 | 0.529 | 0.30 ÷ 0.90 | 7.2 |
| 50 | 0.387 | 0.391 | 0.30 ÷ 0.90 | 8.3 |
| 70 | 0.268 | 0.270 | 0.30 ÷ 0.90 | 10.0 |
| 95 | 0.193 | 0.195 | 0.30 ÷ 0.90 | 11.5 |
| 120 | 0.153 | 0.154 | 0.30 ÷ 0.90 | 13.0 |
| 150 | 0.124 | 0.126 | 0.30 ÷ 0.90 | 14.3 |
| 185 | 0.0991 | 0.100 | 0.30 ÷ 0.90 | 16.2 |
| 240 | 0.0754 | 0.0762 | 0.30 ÷ 0.90 | 18.7 |
| 300 | 0.0601 | 0.0607 | 0.30 ÷ 0.90 | 21.0 |

## Claims

1. A flexible electric multiple elementary wire cable including multiple elementary wires made of red copper or tinned copper, **characterized in that** the conductor of said cable has the following constructional parameters, for the disclosed cross-sections:
| | **CHARACTERISTICS OF THE INVENTIVE FLEXIBLE ELECTRIC CABLE** | | | |
|---|---|---|---|---|
| | 1 | | 2 | 3 |
| Cross Section of the conductor [mm²] | Maximum electric resistance [at 20°C] of the conductor | | Diameter of the used elementary wires [mm] | Maximum diameter of the conductor [mm] |
| | Red Copper [Ohm/km] | Tinned Copper [Ohm/km] | | |
| 6 | 3.08 | 3.11 | 0.30 ÷ 0.90 | 3.2 |
| 10 | 1.83 | 1.84 | 0.30 ÷ 0.90 | 3.8 |
| 16 | 1.15 | 1.16 | 0.30 ÷ 0.90 | 4.9 |
| 25 | 0.727 | 0.734 | 0.30 ÷ 0.90 | 6.1 |
| 35 | 0.524 | 0.529 | 0.30 ÷ 0.90 | 7.2 |
| 50 | 0.387 | 0.391 | 0.30 ÷ 0.90 | 8.3 |
| 70 | 0.268 | 0.270 | 0.30 ÷ 0.90 | 10.0 |
| 95 | 0.193 | 0.195 | 0:30 ÷ 0.90 | 11.5 |
| 120 | 0.153 | 0.154 | 0.30 ÷ 0.90 | 13.0 |
| 150 | 0.124 | 0.126 | 0.30 ÷ 0.90 | 14.3 |
| 185 | 0.0991 | 0.100 | 0.30 ÷ 0.90 | 16.2 |
| 240 | 0.0754 | 0.0762 | 0.30 ÷ 0.90 | 18.7 |
| 300 | 0.0601 | 0.0607 | 0.30 ÷ 0.90 | 21.0 |
thereby said conductor has both a flexibility equal to or better than the flexibility of electric multiple elementary wire conductors of Class 5 of the IEC 60228 standard and an electric resistance meeting the electric resistance requirements of electric multiple elementary conductors of Class 2 of said IEC 60288 standard.

2. An electric cable, according to claim 1, **characterized in that** said conductor has a cross-section from 6 to 300 mm² and a diameter from 3.2 to 21.0 mm, and each said elementary wire of said cable having a diameter from 0.30 to 0.90 mm, depending on a cross section of each said elementary wire.

## Patentansprüche

1. Flexibles elektrisches Mehrfachelementdrahtkabel, das mehrere Elementdrähte aus rotem Kupfer oder verzinntem Kupfer enthält, **dadurch gekennzeichnet, dass** der Leiter des Kabels die folgenden Konstruktionsparameter für die offenbarten Querschnitte aufweist:
| | KENNGRÖSSEN DES ERFINDUNGSGEMÄSSEN FLEXIBLEN ELEKTRISCHEN KABELS | | | |
|---|---|---|---|---|
| | 1 | | 2 | 3 |
| Querschnitt des Leiters [mm²] | Maximaler elektrischer Widerstand des Leiters [bei 20°C] | | Durchmesser der verwendeten Elementdrähte [mm] | Maximaldurchmesser des Leiters [mm] |
| | Rotes Kupfer [Ω/km] | Verzinntes Kupfer [Ω/km] | | |
| 6 | 3.08 | 3.11 | 0.30 ÷ 0.90 | 3.2 |
| 10 | 1.83 | 1.84 | 0.30 ÷ 0.90 | 3.8 |
| 16 | 1.15 | 1.16 | 0.30 ÷ 0.90 | 4.9 |
| 25 | 0.727 | 0.734 | 0.30 ÷ 0.90 | 6.1 |
| 35 | 0.524 | 0.529 | 0.30 ÷ 0.90 | 7.2 |
| 50 | 0.387 | 0.391 | 0.30 ÷ 0.90 | 8.3 |
| 70 | 0.268 | 0.270 | 0.30 ÷ 0.90 | 10.0 |
| 95 | 0.193 | 0.195 | 0.30 ÷ 0.90 | 11.5 |
| 120 | 0.153 | 0.154 | 0.30 ÷ 0.90 | 13.0 |
| 150 | 0.124 | 0.126 | 0.30 ÷ 0.90 | 14.3 |
| 185 | 0.0991 | 0.100 | 0.30 ÷ 0.90 | 16.2 |
| 240 | 0.0754 | 0.0762 | 0.30 ÷ 0.90 | 18.7 |
| 300 | 0.0601 | 0.0607 | 0.30 ÷ 0.90 | 21.0 |
**dadurch** weist der Leiter sowohl eine Flexibilität gleich der oder besser als die Flexibilität des elektrischen Mehrfachelementdrahtleiters der Klasse 5 des Standards IEC 60228 und einen elektrischen Widerstand auf, der die Anforderungen an den elektrischen Widerstand des elektrischen Mehrfachelementleiters der Klasse 2 des besagten Standards IEC 60288 erfüllt.

2. Elektrisches Kabel nach Anspruch 1, **dadurch gekennzeichnet, dass** der Leiter einen Querschnitt von 6 bis 300 mm² und einen Durchmesser von 3,2 bis 21,0 mm aufweist und dass jeder Elementdraht des Kabels in Abhängigkeit von einem Querschnitt eines jeden Elementdrahtes einen Durchmesser von 0,30 bis 0,90 mm aufweist.

## Revendications

1. Câble électrique souple à fils élémentaires multiples comportant des fils élémentaires multiples constitués de cuivre rouge ou de cuivre étamé, **caractérisé en ce que** le conducteur dudit câble possède les paramètres de construction suivants, pour les sections décrites :
| | CARACTERISTIQUES DU CABLE ELECTRIQUE SOUPLE DE L'INVENTION | | | |
|---|---|---|---|---|
| | 1 | | 2 | 3 |
| Section du conducteur [mm²] | Résistance électrique maximum [à 20 °C] du conducteur | | Diamètre des fils élémentaires utilisés [mm] | Diamètre maximum du conducteur [mm] |
| | Cuivre Rouge [Ohm/km] | Cuivre Etamé [Ohm/km] | | |
| 6 | 3,08 | 3,11 | 0,30 ÷ 0,90 | 3,2 |
| 10 | 1,83 | 1,84 | 0,30 ÷ 0,90 | 3,8 |
| 16 | 1,15 | 1,16 | 0,30 ÷ 0,90 | 4,9 |
| 25 | 0,727 | 0,734 | 0,30 ÷ 0,90 | 6,1 |
| 35 | 0,524 | 0,529 | 0,30 ÷ 0,90 | 7,2 |
| 50 | 0,387 | 0,391 | 0,30 ÷ 0,90 | 8,3 |
| 70 | 0,268 | 0,270 | 0,30 ÷ 0,90 | 10,0 |
| 95 | 0,193 | 0,195 | 0,30 ÷ 0,90 | 11, 5 |
| 120 | 0,153 | 0,154 | 0,30 ÷ 0,90 | 13,0 |
| 150 | 0,124 | 0,126 | 0,30 ÷ 0,90 | 14,3 |
| 185 | 0,0991 | 0,100 | 0,30 ÷ 0,90 | 16,2 |
| 240 | 0,0754 | 0,0762 | 0,30 ÷ 0,90 | 18,7 |
| 300 | 0,0601 | 0,0607 | 0,30 ÷ 0,90 | 21,0 |
grâce à quoi ledit conducteur présente à la fois une souplesse égale ou supérieure à la souplesse des fils électriques conducteurs élémentaires multiples de Classe 5 de la norme IEC 60228 et une résistance électrique conforme aux exigences de résistance électrique des conducteurs électriques élémentaires multiples de Classe 2 de ladite norme IEC 60228.

2. Câble électrique, selon la revendication 1, **caractérisé en ce que** ledit conducteur présente une section comprise entre 6 et 300 mm² et un diamètre compris entre 3,2 et 21,0 mm, et **en ce que** chaque dit fil élémentaire dudit câble présente un diamètre compris entre 0,30 et 0,90 mm, en fonction d'une section de chaque dit fil élémentaire.
